

Jan. 5, 1971

M. G. KINNAVY

3,552,175

METHODS OF PERMANENTLY ELONGATING STRIP

Filed Feb. 28, 1968

3 Sheets-Sheet 1

Fig. 1.



Fig. 2.

Idealized Stress - Strain Diagram



Fig. 3.

Yield on Tension Side of Strip



Fig. 4.

Yield on Both Sides of Strip



INVENTOR

Martin G. Kinnavy

By  
Gedel, Stock & Eisenhauer  
his attorney

Jan. 5, 1971

M. G. KINNAVY

3,552,175

METHODS OF PERMANENTLY ELONGATING STRIP

Filed Feb. 28, 1968

3 Sheets-Sheet 2

Fig. 5. Strip Elongation Upon Bending Strain Reversal



Fig. 6. Strip Elongation Upon Bending Strain Reversal



Fig. 7. Graph Showing Different Regions of Elongation & Bending Strain Parameters.



INVENTOR

Martin G. Kinnavy

*Duwell, Kinnavy & Greenbaum  
is attorney's*

Jan. 5, 1971

M. G. KINNAVY

3,552,175

METHODS OF PERMANENTLY ELONGATING STRIP

Filed Feb. 28, 1968

3 Sheets-Sheet 3

Fig. 8.



Fig. 9. Table I Summary of Method

| Criterion | Tension Force                                                                               | Incremental Elongation                                               | Strain                                                                                                    |
|-----------|---------------------------------------------------------------------------------------------|----------------------------------------------------------------------|-----------------------------------------------------------------------------------------------------------|
| Case IA   | $\frac{1}{2\beta} \geq 1 - \frac{F}{\sigma_y t}$                                            | $\frac{F}{\sigma_y t} = 1 - \frac{1}{4\beta} (1 + \beta - \alpha)^2$ | $\Delta e = \left[ 2\beta - \sqrt{8\beta(1 - \frac{F}{\sigma_y t})} \right] \epsilon_y$                   |
| Case IB   | $\frac{1}{2}(1 - \frac{F}{\sigma_y t}) \leq \frac{1}{2\beta} \leq 1 - \frac{F}{\sigma_y t}$ | $\frac{F}{\sigma_y t} = 1 - \frac{1}{4\beta} (1 + \beta - \alpha)^2$ | $\Delta e = \left( \frac{F}{R\sigma_y \epsilon_y} - 1 \right) \epsilon_y$                                 |
| Case II   | $\frac{1}{2\beta} \leq \frac{1}{2} (1 - \frac{F}{\sigma_y t})$                              | $\frac{F}{\sigma_y t} = \frac{\alpha}{\beta}$                        | $\Delta e = \left( \frac{F}{R\sigma_y \epsilon_y} - 1 \right) \epsilon_y$<br>$= (2\alpha - 1) \epsilon_y$ |

INVENTOR

Martin G. Kinnavy

*Martin G. Kinnavy  
Gould, Shulman & Lissner  
his attorneys*

## 1

3,552,175

METHODS OF PERMANENTLY  
ELONGATING STRIP

Martin G. Kinnavy, Warren, Ohio, assignor, by mesne assignments, of 40/90 interest to Richard W. Herr, Cortland, Ohio; 15/90 interest to Salem Corporation, Carnegie, Pa., a corporation of Pennsylvania; and 35/90 interest to a Trust whose trustees are Richard W. Herr and Jean L. Herr, both of Cortland, Ohio, The Union Savings & Trust Company, Warren, Ohio, and John U. Anderson, Jr., Pittsburgh, Pa.

Filed Feb. 28, 1968, Ser. No. 708,947  
Int. Cl. B21d 11/02

U.S. Cl. 72—296

10 Claims

## ABSTRACT OF THE DISCLOSURE

A strip is permanently elongated by applying a tension force to it and constraining it while under tension to at least one bend and at least one bend reversal which causes yielding and an incremental elongation strain that is produced between a bend and a subsequent bend reversal in which the magnitude of incremental elongation strain is related to the applied tension force and the applied bending strains.

This invention relates to a method of permanently elongating strip material to remove irregularities in shape and to modify physical properties or structure.

## I. PROBLEM PRESENTED TO THE INVENTOR

The manufacture of metal strip leaves  
irregularities

A common problem in the production of continuous metal strip is the irregularity of shape in the form of wavy edges and bubbles between the edges. For many applications, material with such irregularities is neither saleable nor useable. These irregularities commonly appear in strip produced by established methods and modification of those methods is either not feasible or too costly. The problem of strip irregularities, therefore must be solved in operations subsequent to the basic strip production operations.

## II. PRIOR ART

Stretching process to remove irregularities  
in metal strip

One of the earliest methods for removing irregularities from strip or plate was the simple jaw stretch leveler which dates back to the nineteenth century. If one considers that a metal strip is composed of a plurality of metal fibers running in a plane in the longitudinal direction of a metal strip, then in the case of an elastic-perfectly plastic material, pure stretching with the longest fiber elongated into the yield zone will produce leveled strip; see definitions of leveled strip infra. If on the other hand the same strains are applied to a material which work-hardens, a somewhat different effect takes place. Fibers which were short will remain short fibers in the "stretch-leveled strip." The reason for this is that after all the fibers were strained to the same length with each fiber undergoing a different individual strain, the more highly strained material recovered a greater amount upon unloading. Thus the strip condition is only partially corrected. The consequence of this is that pure stretch leveling (see definition of leveling infra)

## 2

works best on materials which work-harden only to a slight degree; that is, to materials which are nearly elastic-perfectly plastic. For this class of materials, however, stretch leveling is a very easily controlled process in that the only requirement is that the longest fiber be strained to at least the yield point. In view of the necessity to strain the shortest fibers well into the yield zone, the process of stretch leveling is not useful for materials in which the ultimate tensile strain is only nominally higher than the yield strain.

Simple jaw stretcher leveling is applicable only to the stretching of material in sheet form and not to a continuous process. Nevertheless, the idea of simple stretching has been applied to stretching of strip continuously. In this process the essential components are a drag bridle, a drive bridle, a suitably powered mechanical drive system, and the associated controls. While this process, at first glance, embodies the simplicity of the simple jaw stretcher, close examination discloses serious, but not obvious, weaknesses:

(1) It is necessary with continuous stretcher leveling, to provide sufficient tension capability in the power transmission system to produce the full yield tension in any material to be processed. This high tension requirement imposes the requirement of large expensive drive systems.

(2) Basic kinematic analysis of the bridle-strip system shows that almost all of the strip elongation produced in the process must take place while the strip is in contact with the highest tension drag bridle roll. The consequence of this is that the roll covering, usually an elastomeric material, has an abbreviated life. Furthermore, because the strip approaches this roll while still in the elastic stress range and leaves the roll when in the plastic stress range after having been extended an arbitrary amount, there is large unavoidable velocity mismatch between the strip and the roll covering.

(3) In many systems, it has been common to connect the mechanical drive systems of the drag bridle system to the drive bridle system. The reason for this is to eliminate electrical motors and generators. This cost saving, however, is not without penalty. In a completely geared system one has no control over the distribution of the torque supplied to each drive and drag bridle roll because loads and torques always follow the stiffest possible paths. As a result of this, the manufacturers of this equipment have no control of torque distribution. The problem is further complicated by roll cover wear to the extent that even if only one cover wears, all roll covers must be reground. Furthermore, because any bridle roll will change tension, the strain in the strip is correspondingly changed, and thereby produces an additional source of small velocity mismatch which effect cannot (in these systems) be minimized by adjustment of individual motor or generator units.

## Roller leveling process

Another well-known method to level strip is the roller leveling process. This process is applicable to sheet leveling and to continuous strip leveling. It consists of passing the material between two sets of rolls placed relative to each other so that the strip is constrained to a tortuous path, thereby causing flexing of the material in alternate directions. This process is known to level strip. Generally, the work rolls are small in diameter and tend to diminish in size as the strip thickness to be processed is decreased. For example, one manufacturer uses  $\frac{1}{8}$  inch diameter

rolls for a thickness range of 0.010 inch to 0.050 inch and 1½ inch diameter rolls for a thickness range of .015 inch to .064 inch. The use of small work rolls has necessitated that other sets of rolls of approximately twice the diameter of the work rolls be used in support of the work rolls to prevent excessive deflection; hence the so-called four-high leveler consists of two sets of work rolls plus two sets of backup rolls to support the work rolls.

In recent times, even four-high machines have had to become six-high machines because of the deflection problems. While backup rollers and backup rollers for backup rollers have, to a large degree, surmounted the deflection problems, they have introduced a whole new array of process deficiencies. One of the more serious defects is the so-called stripping problem—a direct effect of the backup roll. Another very serious defect is the control problem. It has been common practice to design into roller levelers vertical adjustability of the backup roll system so that tight portions of the strip might be subjected to more work in the process while loose portions of the strip are subjected to less working.

Roller levelers are of two types, driven and non-driven or pull-through. A serious defect associated with the former type is the strip marking caused by the velocity mismatch between the strip and the driven rolls. The velocity mismatch arises as the strip is elongated in the process, and for which no provision is readily made in the roller drive system. Attempts to overcome this operational defect have been made by using adjustable slip clutches in the drive systems, as well as by resorting to other non-positive drive means, e.g. hydraulic drives.

The roller leveler with a skilled operator at the controls can produce acceptable strip from an appearance point of view. However, in many cases, leveled strip is subsequently slit into narrower coils. Because of the differential working of the rolls against the strip, different residual stress patterns exist across the width of the strip. Because of these differential residual stresses, there appears in the plane of the strip another system of stresses which when disturbed by a slitting operation produces objectionable edge bow in the slit coils. To overcome some of the limitations of roller leveling, many machine builders have incorporated tension bridles to the roller leveling process. This has produced an improved product and has allowed the processors to handle strip of lighter gauge than could be leveled without tension.

A well-known process which uses high tension bridles is the Compagnie des Ateliers et Forges de la Loire (C.A.F.L. Process). Another tension roller leveling process known as the BNF process is described in Research Report A1241, dated June 1969 of the British Non-Ferrous Metals Research Association entitled, "The Elimination of Edge Bow in Slit Strip."

#### Shortcomings of the prior art

While all of the foregoing approaches to the leveling process have had varying degrees of success, there remains with all of them serious drawbacks. In every instance in which work rolls are used for the purpose of flexing the strip, that is, in the roller leveling process, the tension roller leveling process, the C.A.F.L. process, and the BNF process, the work rolls are invariably small in diameter and require the use of backup rolls. With small work roll diameters, operating speeds are low, the design is complex because of the need for backup rolls, and there are greater wear and maintenance problems associated with frequent dressing of the work rolls and frequent work roll changes. Furthermore, the use of a backup roll system frequently causes strip marking.

#### III. THE INVENTION PRESENTS A NEW APPROACH TO THE ELONGATION OF STRIP MATERIAL

The present invention is a new process of permanently elongating metal strip. This can be used to remove strip

irregularities or to modify the physical properties of the strip among other uses. For any given set of physical properties of the strip material, one can assign combinations of tension and bending radii such that the desired strip elongation will be produced, and the desired effects, including leveling and modification of physical properties will result. It is possible that an arbitrary combination of tension and bending will produce some elongation. These arbitrary combinations, however, of tension and bending will not produce the result sought whereas the new process will produce the desired result with great accuracy.

Use of the new process avoids major equipment problems encountered in the present methods (prior art) for elongating strip. The advantages of the new process are: low maintenance of equipment, low downtime of equipment, no strip marking caused by the differential velocity between driven rolls and strip, prolonged life of bridle roll covering, relatively low tension requirements, simplicity of control, ease of operation, and no restrictive speed limit. Furthermore because the new process relates tension with radius of curvature of bending in a prescribed manner, one is able to optimize tensions and roll diameter combinations to achieve the desired result. By doing this one is no longer limited to the use of small diameter rolls. This can eliminate the design complexity of a backup roll system as well as the operational difficulties associated with such systems including but not limited to strip marking.

#### Definitions

(1) Leveling.—Leveling is a process by which shape irregularities in metal strip are removed so that the strip appears uniform. Leveling removes wrinkles from strip but not gross irregularities such as coil set or roll set (defined infra). Leveling makes all fibers of equal length in any given plane. The fibers, however, may vary in length from plane to plane throughout the thickness and the strip will still be leveled. The strip may have roll set or coil set and still be leveled.

(2) Leveled strip.—If an area of metal strip without roll or coil set were laid upon a flat table and its surface conformed everywhere with the surface of the table, it would be considered as flat or leveled strip. Irregular strip laid upon a flat table would not be everywhere in contact with the surface of the table. In this case some fibers would be longer than other fibers.

(3) Coil set or roll set.—A distinction must be made between local strip irregularities removable in a leveling process and the strip condition known as roll or coil set. If a length of strip assumes a longitudinal curvature when it is free of restraint, it is said to have roll or coil set. It is possible for a length of strip to have roll set with or without irregularities. Strip with roll or coil set, but without irregularities, is considered herein to be leveled strip. A simple multi-roll flattener can remove coil set from strip, but it generally is incapable of removing strip irregularities. If one considers strip to be comprised of a multitudinous array of fibers, each fiber in flat and leveled strip will have the same length. Strip with coil or roll set will correspond to a linear variation of fiber length throughout the thickness of the strip. If this pattern of variation is identical in a transverse direction, the strip is said to be leveled. If this variation changes in a transverse direction, the strip would have shape irregularities in addition to roll or coil set. Coil or roll set is related to what is called transverse bow by Poisson's Ratio, a physical property of the strip.

I provide a method of permanently elongating strip which comprises, applying a tension force to the strip, and constraining the strip while under tension to at least one bend and at least one bend reversal which causes yielding and an incremental elongation strain that is produced between a bend and a subsequent bend reversal in which the magnitude of incremental elongation strain is related to the applied tension force such that when the yielding occurs on alternate sides of the strip on succes-

sive bends the increment of elongation strain follows the equation

$$\Delta e = \frac{t}{2} \frac{R_1 + R_2}{R_1 R_2} - \sqrt{2tey \frac{R_1 + R_2}{R_1 R_2} \left(1 - \frac{F}{\sigma_y t}\right)}$$

in which

$F$ =tension force per unit width of strip

$\sigma_y$ =tensile yield stress

$t$ =strip thickness

$\epsilon_y$ =tensile yield strain

$\Delta e$ =increment of elongation strain, and

$R_1, R_2$ =radii of successive bends

I provide a method of permanently elongating strip which comprises, applying a tension force to the strip, and constraining the strip while under tension to at least one bend and at least one bend reversal which causes yielding and an incremental elongation strain that is produced between a bend and a subsequent bend reversal in which the magnitude of incremental elongation strain is related to the applied tension force such that when yielding occurs on at least one side of the strip at a bend and on both sides of the strip at the subsequent bend reversal the increment of elongation strain follows the equation

$$\Delta e = \frac{F}{2\sigma_y} \frac{R_1 + R_2}{R_1 R_2} - \epsilon_y$$

in which

$F$ =tension force per unit width of strip

$\sigma_y$ =tensile yield stress

$\epsilon_y$ =tensile yield strain

$\Delta e$ =increment of elongation strain, and

$R_1, R_2$ =radii of successive bends

Other details, objects and advantages of the invention will become apparent as the following description of a present preferred method of practicing the invention proceeds.

In the accompanying drawings I have illustrated a present preferred method of practicing the invention in which:

FIG. 1 is a stress-strain diagram;

FIG. 2 is an idealized stress-strain diagram;

FIG. 3 is a diagram showing yielding on tension side of the strip—known as Case I;

FIG. 4 is a diagram showing yielding on both tension and compression sides of the strip—known as Case II;

FIG. 5 is a diagram of strip elongation upon bending strain reversal—Case II;

FIG. 6 is a diagram of strip elongation upon bending strain reversal—Case I;

FIG. 7 is a diagram showing different regions of elongation and bending strain parameters;

FIG. 8 is a schematic diagram of apparatus used in examples of application of method to strip material; and

FIG. 9 is a table showing incremental elongation strain for Case IA, Case IB and Case II.

Elongation of strip is related to leveling. This relationship can be shown by referring to an idealized stress-strain diagram for an elastic perfectly plastic material as shown in FIG. 1. Consider, for example, irregular strip free of coil set. If the strip is irregular, it has bubbles or waves and there will be a difference in fiber length. If a length of such strip is elongated, the short fibers will be loaded in tension first. As the elongation increases, longer fibers will begin to share the tension load. If the elongation is further continued until the longest fiber is strained beyond the yield point, the shortest fiber will be strained to an even greater magnitude. However, each fiber so elongated will have the same stress. This is illustrated in FIG. 1 in which Point 1 shows the stress and strain for the longest fiber, and Point 2 shows the stress and strain for the shortest fiber. Now, if the strip is un-

loaded, each fiber will relax the same amount because the path of the stress-strain points is parallel to the initial elastic loading curve. This means that recovery strain  $R_1$  is equal to recovery strain  $R_2$ . Thus the final condition of the strip will be such that every fiber has the same length and the strip is said to be leveled.

Consider a material in which work-hardening takes place after the yield point is reached. If such a material is elongated in a similar way, we will produce stress-strain Points 3 and 4, as shown. Now, if the load is relaxed, it can be seen that the recovery strain for the longest fiber  $R_3$  is less than the recovery strain for the shortest fiber  $R_4$ . In this case the strip condition, although it can be improved, can only be partially corrected. Thus leveling by means of stretching or elongating the material works best on materials which do not exhibit a high degree of work-hardening. For materials with little or no work-hardening, leveling through stretching is a very easily controlled process in that the only requirement is that the longest fiber be strained at least to the yield point. Thus the problem of leveling becomes the establishment of a suitable mechanical process whereby all fibers of the strip are stretched beyond the yield point. The amount of stretch or elongation necessary to level strip depends upon the initial fiber length variation throughout the strip.

In the bending of strip, straight lines in an unloaded, unstrained strip will remain straight upon the deflection which accompanies the application of loads. These straight lines, however, will become inclined toward each other. The consequence of this is that some fibers of the strip will elongate with respect to other fibers of the strip, and the relative elongation will be proportional to the distance from the unstrained fiber; that is, the fiber strain is proportional to the distance from the unstrained, or neutral, fiber. This may also be stated in another way, namely; the fiber strain is a linear function of its distance from the neutral fiber.

Consider, now, the idealized stress-strain diagram shown in FIG. 2 in which stress is the ordinate, and strain is the abscissa. In this diagram, Point 1 is the yield point in tension, and Point 2 is the yield point in compression. The magnitude of the tensile yield stress has been taken as equal to the magnitude of a compressive yield stress. The yield strains in both tension and compression have also been taken as equal. If tension is applied to a fiber, it will be accompanied by a strain such that all stress-strain points will lie upon the straight line 0-1 until the yield stress is reached. Thereafter, as the strain is increased, the stress will remain the same and all stress-strain points after yielding will lie upon the line 1-5.

If a fiber has been strained such that its stress and strain are given by Point 3 in FIG. 2, a further increase in strain produces no increase in stress. On the other hand, if the strain at Point 3 is reduced, the stress will decrease so that all stress-strain points upon continued decreasing strain will lie along the line 3-4 which line is parallel to the initial elastic stress-strain line. Thus Point 4 may have a positive strain and a negative or compressive stress. If a further strain decrease takes place, the stress-strain path will continue leftward along the line defined by 2-6. Thus, with the model shown, it is possible to develop an infinite number of continuous stress-strain paths bound by extensions of the tensile yield stress line 1-5 and the compressive yield stress line 2-6. Any stress-strain path from one of these lines to the other will always be parallel to the initial elastic curve.

Consider typical linear strain distributions and their associated stress distributions through the strip thickness. It is necessary to distinguish between stress distributions in which the yield stress appears on either one or both sides of the strip. If the yield stress is reached in tension alone, this is a Case I stress distribution. If the yield stress value is reached on both tension and compression sides

of the strip, it is called a Case II stress distribution. Refer to FIGS. 3 and 4.

As a consequence of the linear strain distribution, any strain distribution may be considered to consist of an elongation component and a bending component. The elongation component is the strain that exists at the middle of the strip; the bending component is zero at the middle of the strip and is maximum at the surface of the strip. Strain components are designated in terms of the yield strain  $\epsilon_y$ . Thus  $\alpha\epsilon_y$  is the extension component of the strain and  $\beta\epsilon_y$  is the bending component of the strain. Two strain distributions are shown on the lefthand sides of FIGS. 3 and 4 in which the vertical line is taken as the zero strain axis, and strains to the right of this line are taken as tension strains.

The stress distributions corresponding to these strain distributions are obtained by utilizing the stress-strain diagram, FIG. 2, together with the strain distributions shown. These stress distributions are shown at the righthand sides of FIGS. 3 and 4. The force per unit width of strip corresponding to the Case I stress distribution will be given by

$$F = \sigma_y t \left[ 1 - \frac{1}{4\beta} (1 + \beta - \alpha)^2 \right] \quad 25$$

A similar calculation for the Case II stress distribution will show that the tension force per unit width of the strip will be given by

$$F = \sigma_y t \frac{\alpha}{\beta}$$

The geometrical relation between bending strain and curvature is given by

$$\beta\epsilon_y = \frac{t}{2R}$$

where  $R$  is the radius of curvature of the neutral fiber of the strip.

With these established preliminary considerations, the strip subjected to tension in combination with a bending strain will be examined when it is subjected to a reversal of the bending strain when the combination of tension and bending strains lies within the teaching of this invention.

FIG. 5 shows a strain distribution by means of the line at the left side of the figure, this line labeled 1. The surfaces of the strip are indicated by the horizontal lines at the top and bottom of the figure and the middle fiber of the strip is so labeled. The initial strain distribution is made up of the extension or elongation strain component,  $\alpha\epsilon_y = 1.25 \epsilon_y$  and the bending strain component,  $\beta\epsilon_y = 2.50\epsilon_y$ . The stress distribution which corresponds to this strain distribution is obtained through use of the stress-strain diagram FIG. 2, and is shown at the right of FIG. 5 by the series of straight lines 0-1-1\*-1-1-0. This stress distribution is in equilibrium with the force per unit width of strip  $F = 0.5 \sigma_y t$ .

Now upon reversal of the bending strain component, the slope of the strain distribution is simply reversed but since the applied load remains the same the new stress distribution must be in equilibrium with the same force; namely,  $F = 0.5 \sigma_y t$ . The constraints of the stress-strain relations described earlier and illustrated in FIG. 2 must be followed. The only strain distribution that has the prescribed bending strain component that obeys the stress-strain constraints described, and that transforms the initial stress distribution into a new stress distribution in equilibrium with the applied tension force, is the strain distribution labeled 2. The new stress distribution is given by 0-2-2-2\*-2-0. Upon inspection one will see that a point

$$\frac{F}{\sigma_y t} \frac{t}{2}$$

above the middle fiber, a strain change of  $\epsilon_y$  occurs, while

at Point 2\* no strain change occurs. Point 2\* is located at a distance

$$\frac{F}{\sigma_y t} \frac{t}{2} - \frac{1}{2\beta} \frac{t}{2}$$

above the middle fiber. It now follows directly from geometry that the increment of elongation strain of the middle fiber,  $\Delta e$  is

$$\Delta e = \left( \frac{F}{\sigma_y t} 2\beta - 1 \right) \epsilon_y \quad 10$$

Use of the earlier stated geometrical relation between bending strain, strip thickness, and radius of curvature in this equation yields a more useful expression for the incremental strain produced during bending strain reversal under maintained tension, namely,

$$\Delta e = \left( \frac{F}{R\sigma_y} - 1 \right) \epsilon_y \quad 20$$

From this equation an expression for force required to produce a given increment of elongation strain may be obtained, namely,

$$F = R\sigma_y \epsilon_y \left( \frac{\Delta e}{\epsilon_y} + 1 \right) \quad 25$$

or

$$F = (\gamma + 1) \frac{R\sigma_y^2}{E} \quad 30$$

in which

$$\gamma = \frac{\Delta e}{\epsilon_y}$$

It is of significance that the increment of elongation strain is independent of strip thickness. This result is of utmost importance. However, as the material thickness is reduced, a given tension force causes increasing stresses. The particular case of strip thickness approaching zero indicates a tendency toward infinite stresses which cannot exist. The explanation of this apparent anomaly lies in the range of validity of the above expression. A condition that must be met for this expression to apply is

$$\frac{R\epsilon_y}{t} \leq 1 - \frac{F}{\sigma_y t} \quad 45$$

or equivalently

$$t \geq R\epsilon_y + \frac{F}{\sigma_y} \quad 50$$

The above teaching was directed to the case of a stress distribution which has been designated a Case II stress distribution. The effect of a bending strain reversal when a Case I stress distribution exists in the strip will now be considered. In FIG. 6 a selected extension strain component of  $\alpha\epsilon_y = 1.25 \epsilon_y$  and a bending strain component of  $\beta\epsilon_y = 1.50 \epsilon_y$  are used.

The reversal of the bending strain must be accomplished within the same constraints as before. In this case, it can be observed that the stress change at the surface initially at the tension yield stress is

$$2\sigma_y \sqrt{2\beta \left( 1 - \frac{F}{\sigma_y t} \right)}$$

and that the stress and strain remain unchanged at a point a distance above the middle fiber given by

$$\frac{t}{2} \left[ 1 - \sqrt{\frac{2}{\beta} \left( 1 - \frac{F}{\sigma_y t} \right)} \right] \quad 70$$

The strain change at the surface initially strained above the yield strain in tension is

$$2\epsilon_y \sqrt{2\beta \left( 1 - \frac{F}{\sigma_y t} \right)} \quad 75$$

From geometry, the incremental elongation strain of the middle fiber is

$$\Delta e = \left[ 2\beta - \sqrt{8\beta \left( 1 - \frac{F}{\sigma y t} \right)} \right] \epsilon y$$

which upon use of the earlier shown expression for bending strain becomes

$$\Delta e = \left[ \frac{t}{Rey} - \sqrt{\frac{4t}{Rey} \left( 1 - \frac{F}{\sigma y t} \right)} \right] \epsilon y$$

This expression is valid for all surface strain changes given by

$$2\epsilon y \sqrt{2\beta \left( 1 - \frac{F}{\sigma y t} \right)} \leq 2\epsilon y$$

which is equivalent to

$$\frac{Rey}{t} \geq 1 - \frac{F}{\sigma y t}$$

One may elect to subject the strip while under tension to bending strains and bending strain reversals such that the radii of curvature corresponding to those bending strains and bending strain reversals are unequal, in which case the increments of elongation strains produced during bending strain reversals are

$$\Delta e = \left[ \frac{F}{2\sigma y e y} \frac{R_1 + R_2}{R_1 R_2} - 1 \right] \epsilon y$$

when

$$\frac{2\epsilon y}{t} \frac{R_1 + R_2}{R_1 R_2} \leq 1 - \frac{F}{\sigma y t}$$

and

$$\Delta e = \frac{t}{2} \frac{R_1 + R_2}{R_1 R_2} - \sqrt{2\epsilon y \frac{R_1 + R_2}{R_1 R_2} \left( 1 - \frac{F}{\sigma y t} \right)}$$

when

$$\frac{2\epsilon y}{t} \frac{R_1 + R_2}{R_1 R_2} \geq 1 - \frac{F}{\sigma y t}$$

The stress distributions at a bend and at a bend reversal falling within the teaching of this invention are simple, that is, the only stresses below the yield stress in magnitude are confined to a region of the strip thickness and the stresses in this region vary linearly and continuously from the maximum tension value to the maximum compression value. All stress distributions, however, that prevail between a given bend and a subsequent bend reversal are not simple. But within the teaching herein, the process relates to the extension of strip that occurs while subjected to a tension force from a simple stress distribution which is associated with a bending strain, to a subsequent simple stress distribution, which is associated with a bending strain of opposite sign. In these instances the previous strain history will not be evident in the stress distribution; however the slope of the elastic portion of the stress distribution will not be the same as the slope of the strain distribution.

In order that stress distributions of the Case II type remain simple, it is necessary that Point 2\* in FIG. 5 be above Point 1\*. For this to be so

$$\frac{F}{\sigma y t} \frac{t}{2} - \frac{\sigma y t}{4\beta \sigma y} \geq -\frac{F}{\sigma y t} \frac{t}{2} + \frac{\sigma y t}{2\beta \sigma y}$$

or

$$\frac{F}{\sigma y t} \frac{t}{2} - \frac{3}{2} \frac{Rey}{t} \geq 3 \frac{Rey}{t}$$

It has been found convenient to use the variables  $\alpha$  and  $\beta$  described earlier in the application of the method to prac-

tical problems. With the substitution of these variables in the expression above, we have

$$\alpha \geq \frac{3}{4}$$

In the equation

$$F = (\gamma + 1) \frac{Rey^2}{E}$$

the above limitation on  $\alpha$  imposes a restriction on  $\gamma$ , namely,  $\gamma \geq 0.5$ .

Similarly for simple Case I stress distributions to transform into simple Case I stress distributions upon the reversal of the bending strain, hereafter called a Case IA stress distribution, the requirement is

$$\alpha \geq 1 - \frac{\sqrt{2} - 1}{\sqrt{2} + 1} \beta$$

(Case IA)

20 In some cases, a simple Case I stress distribution is transformed into a simple Case II stress distribution, hereafter called a Case IB stress distribution, and the condition for this is that

$$\alpha \geq \frac{3}{2} - \frac{F}{\sigma y t} \beta$$

(Case IB)

or equivalently,

$$\alpha \geq \frac{3}{2} - \frac{F}{2R\sigma y e y}$$

(Case II)

The above conditions have been illustrated graphically in FIG. 7. We have shown that for both Case II and Case IA the increment of elongation strain described earlier is given by

$$\Delta e = \left( \frac{F}{R\sigma y e y} - 1 \right) \epsilon y$$

and that for Case I-A the increment of elongation strain is given by

$$\Delta e = \left[ \frac{t}{Rey} - \sqrt{\frac{4t}{Rey} \left( 1 - \frac{F}{\sigma y t} \right)} \right] \epsilon y$$

or equivalently,

$$\Delta e = \left[ 2\beta - \sqrt{8\beta \left( 1 - \frac{F}{\sigma y t} \right)} \right] \epsilon y$$

The invention can also be understood by practical applications of the method to strip material under certain conditions as shown by the following examples. The apparatus (referring to FIG. 8) used in these examples consisted essentially of a means to apply a tension force to the strip and a means to produce bending strains and bending strain reversals. The means of applying tension force was a hydraulic cylinder which was connected to a force gage which was connected to one end of the strip. The other end of the strip was connected to a force gage which was connected by a bracket to a fixed building column. Bending strains were applied by means of rolls carried on a cart riding on a smooth track. A hydraulic power supply was used to provide a source of hydraulic pressure for the hydraulic cylinder. Strip was threaded over and under the rolls mounted on the cart and clamped as shown in FIG. 8. The hydraulic cylinder is used to remove slack from the strip; then a gage length is marked on the strip (50 inches). A suitable tension force is then applied to the strip by means of the hydraulic cylinder, the magnitude of the tension force being measured by means of load cells. The cart is then moved along the length of the strip, thereby subjecting the strip to an initial bending strain distribution; then to a bending strain reversal; then to a second bending strain reversal. The distance between the gage marks

is measured after the passage of the cart along the strip and this measurement is compared with the original gage length. This comparison then yields the strip elongation; that is,

$$\text{percent elongation} = \frac{\text{final length} - \text{initial length}}{\text{initial length}} \times 100$$

## EXAMPLE 1

Material: Aluminum, 3105H25

Thickness:  $t$ , 0.0319 in. (measured)

Yield stress:  $\sigma_y$ , 26,600 lb./in.<sup>2</sup>

Modulus of elasticity:  $E$ , 8,520,000 lb./in.<sup>2</sup>

Yield strain:  $\epsilon_y$ , 0.00312

Yield tension:  $\sigma_y t$ , 850 lb./in. of width

The diameter of the rolls on the cart was 6 inches; thus the bending strain parameter is calculated as follows:

$$\beta = \frac{t}{2R\epsilon_y} = \frac{(0.0319)}{6(0.0319)} (.00312) = 1.695$$

In this example, a tension force of approximately 75 percent of the yield tension was used; i.e.,  $F = 637.5$  lb./in. of strip width. To establish which Case in FIG. 7 is applicable, Table I (FIG. 9) has been developed. Thus,

$$\frac{1}{2\beta} = 0.295 > (1 - 0.75)$$

which shows a Case IA situation.

First  $\alpha$  is computed from the force equation. Thus,

$$\alpha = 1 + \beta - \sqrt{4\beta \left(1 - \frac{F}{\sigma_y t}\right)}$$

Substitution of numerical values gives

$$\alpha = 1 + 1.695 - \sqrt{6.80(0.25)} = 1.39$$

The increment of elongation strain is then

$$\Delta e = \left[ 2\beta - \sqrt{8\beta \left(1 - \frac{F}{\sigma_y t}\right)} \right] \epsilon_y$$

or

$$\Delta e = [(2)(1.695) - \sqrt{(8)(1.695)(0.25)}] = 1.55\epsilon_y$$

In the example fixture the initial bending strain is followed by two bending strain reversals. Thus from the initial bend there is a middle fiber strain of  $\alpha\epsilon_y = 1.39\epsilon_y$  and from the two bending strain reversals, two increments of strain each of magnitude  $\Delta e = 1.55\epsilon_y$  to produce a total elongation strain of

$$\epsilon = [1.39 + (2)(1.55)](.00312) = 0.0140$$

The example result showed that with a gage length of 50 inches an elongation of 0.782 inch was produced, which corresponds to a strain of

$$\epsilon = \frac{0.782}{50} = 0.01564$$

The difference is  $0.01564 - 0.0140$  or 0.00164 or 10.5%.

## EXAMPLE 2

Material: Aluminum, 5052H32

Thickness:  $t$ , 0.040 inch

Yield stress:  $\sigma_y$ , 27,600 lb./in.<sup>2</sup>

Modulus of elasticity:  $E$ , 9,550,000 lb./in.<sup>2</sup>

Yield strain:  $\epsilon_y$ , 0.00288

Yield tension:  $\sigma_y t$ , 1105 lb./in. of width

In this test the bending strain parameter is

$$\beta = \frac{0.040}{(6.040)} (.00288) = 2.30$$

With an applied tension force of  $F = 857$  lb./in. of width,

$$1 - \frac{F}{\sigma_y t} = 1 - \frac{857}{1105} = 0.225$$

and

$$\frac{1}{2} \left(1 - \frac{F}{\sigma_y t}\right) = 0.1125$$

The quantity  $1/2\beta$  is 0.2175 which means a Case IB situation. Thus  $\alpha$  is computed as follows:

$$\alpha = 1 + \beta - \sqrt{4\beta \left(1 - \frac{F}{\sigma_y t}\right)} \\ = 1 + 2.30 - \sqrt{9.2(0.225)} = 1.86$$

15 The increment of elongation strain upon bending strain reversal is

$$\Delta e = \left( \frac{F}{R\sigma_y \epsilon_y} - 1 \right) \epsilon_y = \left( \frac{857}{(3.02)(27600)(.00288)} - 1 \right) \epsilon_y \\ 20 = 2.57\epsilon_y$$

The total elongation strain is obtained as before

$$\epsilon = [1.86 + (2)(2.57)](.00288) \\ = 0.0216$$

25 The test result showed an elongation strain of 0.0222. The difference is 0.0006 or 2.7%.

## EXAMPLE 3

30 Material: Aluminum, 5052H32

Thickness:  $t$ , 0.0512 inch

Yield stress:  $\sigma_y$ , 24,700 lb./in.<sup>2</sup>

Modulus of elasticity:  $E$ , 8,970,000 lb./in.<sup>2</sup>

Yield strain:  $\epsilon_y$ , 0.00276

Yield tension:  $\sigma_y t$ , 1263 lb./in. of width

35 The bending strain parameter is

$$\beta = \frac{0.0512}{(6.0512)} (.00276) = 3.06$$

40 and

$$1/2\beta = 0.1635$$

With a tension force of 653 lb./in. of strip width;

$$1 - \frac{F}{\sigma_y t} = 1 - \frac{653}{1263} = 0.483$$

and

$$\frac{1}{2} \left(1 - \frac{F}{\sigma_y t}\right) = 0.242$$

50 Since

$$\frac{1}{2\beta} < \frac{1}{2} \left(1 - \frac{F}{\sigma_y t}\right)$$

55 it follows from Table I that we have a Case II situation. Thus

$$\alpha = \frac{F}{\sigma_y t} \beta = (0.517)(3.06) = 1.58$$

60 and the increment of elongation strain upon bending strain reversal is

$$\Delta e = (2\alpha - 1)\epsilon_y = 2.16\epsilon_y$$

The total elongation strain is then

$$65 \epsilon = [1.58 + (2)(2.16)](.00276) \\ = 0.0163$$

The observed elongation strain in the experiment was 0.0164 which is different by only 0.6 percent.

70 While I have shown and described a present preferred embodiment of the invention and have illustrated present preferred methods of practicing the same, it is to be distinctly understood that the invention is not limited thereto but may be practiced within the scope of the following claims.

I claim:

1. A method of permanently elongating strip which comprises:

- (a) applying a tension force to the strip; and
- (b) constraining the strip while under tension to at least one bend and at least one bend reversal which causes yielding and an incremental elongation strain that is produced between a bend and a subsequent bend reversal in which the magnitude of incremental elongation strain is related to the applied tension force such:

- (1) that when the yielding occurs on alternate sides of the strip on successive bends the increment of elongation strain follows the equation

$$\Delta e = \frac{t}{2} \frac{R_1 + R_2}{R_1 R_2} - \sqrt{2tey \frac{R_1 + R_2}{R_1 R_2} \left(1 - \frac{F}{\sigma y t}\right)}$$

and

- (2) when yielding occurs on at least one side of the strip at a bend and on both sides of the strip at the subsequent bend reversal the increment of the increment of elongation strain follows the equation

$$\Delta e = \frac{F}{2\sigma y} \frac{R_1 + R_2}{R_1 R_2} - \epsilon y$$

in which

$F$ =tension force per unit width of strip

$t$ =strip thickness

$\sigma y$ =tensile yield stress

$\epsilon y$ =tensile yield strain

$\Delta e$ =increment of elongation strain, and

$R_1, R_2$ =radii of successive bends.

2. A method of permanently elongating strip which comprises:

- (a) applying a tension force to the strip; and
- (b) constraining the strip while under tension to at least one bend and at least one bend reversal which causes yielding and an incremental elongation strain that is produced between a bend and a subsequent bend reversal in which the magnitude of incremental elongation strain is related to the applied tension force such that when the yielding occurs on alternate sides of the strip on successive bends the increment of elongation strain follows the equation

$$\Delta e = \frac{t}{2} \frac{R_1 + R_2}{R_1 R_2} - \sqrt{2tey \frac{R_1 + R_2}{R_1 R_2} \left(1 - \frac{F}{\sigma y t}\right)}$$

in which

$F$ =tension force per unit width of strip

$\sigma y$ =tensile yield stress

$t$ =strip thickness

$\epsilon y$ =tensile yield strain

$\Delta e$ =increment of elongation strain, and

$R_1, R_2$ =radii of successive bends.

3. A method of permanently elongating strip which comprises:

- (a) applying a tension force to the strip; and
- (b) constraining the strip while under tension to at least one bend and at least one bend reversal which causes yielding and an incremental elongation strain that is produced between a bend and a subsequent bend reversal in which the magnitude of incremental elongation strain is related to the applied tension force such that when yielding occurs on at least one side of the strip at a bend and on both sides of the

strip at the subsequent bend reversal the increment of elongation strain follows the equation

$$\Delta e = \frac{F}{2\sigma y} \frac{R_1 + R_2}{R_1 R_2} - \epsilon y$$

in which

$F$ =tension force per unit width of strip

$\sigma y$ =tensile yield stress

$\epsilon y$ =tensile yield strain

$\Delta e$ =increment of elongation strain, and

$R_1, R_2$ =radii of successive bends.

4. A method of permanently elongating strip which comprises:

- (a) applying a tension force to the strip; and
- (b) constraining the strip while under tension to at least one bend and at least one bend reversal which causes yielding and incremental elongation strain that is produced between a bend and a subsequent bend reversal in which the magnitude of incremental elongation strain is related to the applied tension force such that when

$$\frac{2\epsilon y}{t} \frac{R_1 R_2}{R_1 + R_2} \geq 1 - \frac{F}{\sigma y t}$$

the increment of elongation strain follows the equation

$$\Delta e = \frac{t}{2} \frac{R_1 + R_2}{R_1 R_2} - \sqrt{2tey \frac{R_1 + R_2}{R_1 R_2} \left(1 - \frac{F}{\sigma y t}\right)}$$

in which

$\epsilon y$ =yield strain

$t$ =strip thickness

$R_1$ =radius of bend

$R_2$ =radius of succeeding bend

$F$ =tension force per unit width of strip

$\sigma y$ =yield stress.

5. A method of permanently elongating strip which comprises:

- (a) applying a tension force to the strip; and
- (b) constraining the strip while under tension to at least one bend and at least one bend reversal which causes yielding and incremental elongation strain that is produced between a bend and a subsequent bend reversal in which the magnitude of incremental elongation strain is related to the applied tension force such that when

$$\frac{2\epsilon y}{t} \frac{R_1 R_2}{R_1 + R_2} \leq 1 - \frac{F}{\sigma y t}$$

the increment of elongation strain follows the equation

$$\Delta e = \frac{F}{2\sigma y} \frac{R_1 + R_2}{R_1 R_2} - \epsilon y$$

in which

$\epsilon y$ =yield strain

$t$ =strip thickness

$R_1$ =radius of bend

$R_2$ =radius of succeeding bend

$F$ =tension force per unit width of strip

$\sigma y$ =yield stress.

6. A method of permanently elongating strip which comprises:

- (a) applying a tension force to the strip; and
- (b) constraining the strip while under tension to at least one bend and at least one bend reversal which causes an incremental elongation strain that is produced between a bend and a subsequent bend reversal in which the magnitude of incremental strain elongation is related to the applied tension force such that when yielding occurs on only alternate sides of the

strip on successive bends the increment of elongation follows the equation

$$\Delta e = \left[ \frac{t}{Rey} - \sqrt{\frac{4t}{Rey} \left( 1 - \frac{F}{\sigma yt} \right)} \right] \epsilon y \quad 5$$

in which

$\Delta e$ =incremental elongation strain

$t$ =strip thickness

$R$ =radius of bend

$\epsilon y$ =yield strain

$F$ =tension force per unit width of strip

$\sigma y$ =yield stress.

7. A method of permanently elongating strip which comprises:

- (a) applying a tension force to the strip; and
- (b) constraining the strip while under tension to at least one bend and at least one bend reversal which causes an incremental elongation strain that is produced between a bend and a subsequent bend reversal in which the magnitude of incremental strain elongation is related to the applied tension force such that when yielding occurs on one or both sides of the strip at a given bend and on both sides of the strip at the subsequent bend the increment of elongation follows the equation

$$\Delta e = \left( \frac{F}{R\sigma y \epsilon y} - 1 \right) \epsilon y \quad 15$$

in which

$\Delta e$ =incremental elongation strain

$R$ =radius of bend

$\epsilon y$ =yield strain

$F$ =tension force per unit width of strip

$\sigma y$ =yield stress.

8. A method of permanently elongating strip which comprises:

- (a) applying a tension force to the strip; and
- (b) constraining the strip while under tension to at least one bend and at least one bend reversal which causes an incremental elongation strain that is produced between a bend and a subsequent bend reversal in which the magnitude of incremental elongation strain is related to the applied tension force such that when

$$\frac{Rey}{t} \geq 1 - \frac{F}{\sigma yt} \quad 40$$

the increment of elongation follows the equation

$$\Delta e = \left[ \frac{t}{Rey} - \sqrt{\frac{4t}{Rey} \left( 1 - \frac{F}{\sigma yt} \right)} \right] \epsilon y \quad 45$$

in which

$F$ =tension force per unit width of strip

$\sigma y$ =tensile stress

$t$ =strip thickness

$\epsilon y$ =tensile yield strain

$\Delta e$ =incremental elongation, and

$R$ =radius of bend when the bend radius equals the reverse bend radius.

9. A method of permanently elongating strip which comprises:

- (a) applying a tension force to the strip; and
- (b) constraining the strip while under tension to at least one bend and at least one bend reversal which causes an incremental elongation strain that is pro-

duced between a bend and a subsequent bend reversal in which the magnitude of incremental elongation strain is related to the applied tension force such that when

$$\frac{Rey}{t} \leq 1 - \frac{F}{\sigma yt} \quad 5$$

the increment of elongation follows the equation

$$\Delta e = \left( \frac{F}{R\sigma y \epsilon y} - 1 \right) \epsilon y \quad 10$$

in which

$F$ =tension force per width of strip

$\sigma y$ =tensile yield stress

$t$ =strip thickness

$\epsilon y$ =tensile yield strain

$\Delta e$ =incremental elongation, and

$R$ =radius of bend when the bend radius equals the reverse bend radius.

10. A method of permanently elongating strip which comprises:

- (a) applying a tension force to the strip; and
- (b) constraining the strip while under tension to at least one bend and at least one bend reversal which causes yielding and an incremental elongation strain that is produced between a bend and subsequent bend reversal such that for a force of magnitude

$$F = (\gamma + 1) \frac{R\sigma y^2}{E} \quad 20$$

the increment of elongation strain will be  $\Delta e = \gamma \epsilon y$ , in which

$F$ =tension force per unit width of strip

$R$ =bend radius

$\sigma y$ =yield stress

$E$ =modulus of elasticity

$\epsilon y$ =yield strain

$\Delta e$ =increment of elongation strain

$\gamma$ =any numerical coefficient greater than or equal to 0.5.

#### References Cited

##### UNITED STATES PATENTS

|           |         |            |       |        |
|-----------|---------|------------|-------|--------|
| 3,260,093 | 7/1966  | Polakowski | ----- | 72—163 |
| 2,180,879 | 11/1939 | McFadden   | ----- | 72—183 |
| 2,059,993 | 11/1936 | Hanson     | ----- | 72—205 |
| 1,975,846 | 10/1934 | Hartmann   | ----- | 72—164 |

##### FOREIGN PATENTS

|           |        |                |  |
|-----------|--------|----------------|--|
| 1,028,537 | 5/1966 | Great Britain. |  |
| 655,444   | 7/1951 | Great Britain. |  |

##### OTHER REFERENCES

Journal of The Iron and Steel Institute—Batty and Lawson, "Heavy Plate Levellers"; November 1965; pp. 1115—1123.

Iron and Steel Engineer—Bland and Alters; "Tension Leveling"; September 1967; pp. 95—105.

The Magazine of Metals Producing—Kusakabe and Hirasawa; "Shape Improvement of Thin Steel Strip by Using the Roller Stretcher"; December 1967; pp. 93—106.

RICHARD J. HERBST, Primary Examiner

MICHAEL J. KEENAN, Assistant Examiner

U.S. Cl. X.R.

72—160, 205, 316, 378